

## UNITED STATES PATENT OFFICE

CHARLES DANGELMAJER, OF NIAGARA FALLS, NEW YORK, ASSIGNOR, BY MESNE ASSIGNMENTS, TO THE ROESSLER & HASSLACHER CHEMICAL COMPANY, OF NEW YORK, N. Y., A CORPORATION OF DELAWARE

## STABILIZATION OF TRICHLOROETHYLENE

No Drawing.

Application filed January 11, 1929. Serial No. 331,945.

This invention relates to a new composition of matter comprising trichloroethylene and gasoline. The object is to stabilize the trichloroethylene.

One of the difficulties associated with trichloroethylene is its tendency to undergo decomposition during storage and during recovery operations such as distillation. This decomposition is accompanied by the formation of substances of acid character which render the trichloroethylene objectionable for many purposes such as extraction processes and also make it more difficult to store because of the corrosive properties of the decomposition products.

I have discovered that trichloroethylene can be rendered stable for storage and distillation and the development of objectionable degrees of acidity largely avoided by the addition of gasoline or related petroleum hydrocarbons.

I am aware that other stabilizers have been proposed and used, such as xylene, toluene, etc. I have tried these and found that they are not satisfactory primarily because they are not efficient stabilizers and secondarily, because they are more expensive and must be used in larger concentrations than gasoline or other petroleum hydrocarbons.

A few examples will show the stabilizing properties of petroleum hydrocarbons, particularly gasoline.

## Examples

As a measure of the instability of trichloroethylene the acidity of a 25 cc. sample in terms of 0.01 normal sodium hydroxide is used. The indicator is phenolphthalein. Thus, for example, if 25 cc. of a sample requires 10 cc. of 0.01 normal sodium hydroxide solution for complete neutralization its acidity is given as 10.

1. A batch of crude freshly manufactured undistilled trichloroethylene had an original acidity of 0.4, which rose to 300 after storing for 52 days and to much over 1000 after 14 months storage.

2. A portion of the same batch as under 1 was distilled and 0.1% by volume of gasoline was added. The original acidity was

very low and after 52 days was 0.8 and after 14 months it was 4.2.

3. A portion of the same batch as under 1 was distilled and then a few drops of high-acid trichloroethylene was added, also 0.5% by volume of gasoline. After two weeks the acidity was 0.9; after 4 weeks it was 0.7 and after seven weeks it was 0.5. At the end of 14 months the acidity was 2.5.

4. To a batch of crude freshly manufactured undistilled trichloroethylene 0.25% by volume of gasoline was added. A few drops of high-acid unstabilized trichloroethylene was added after distilling the stabilized crude material. The acidity after 2, 4, and 7 weeks and 14 months was 0.6, 0.4, 0.6 and 1.5 respectively.

5. Normal heptane to the extent of 0.25% by volume was added to a batch of trichloroethylene having an initial acidity of 0.6. After 7 months the acidity was unchanged.

6. Ordinary kerosene to the extent of 0.25% by volume was added to trichloroethylene of 0.6 acidity. After seven months there was no change in the acidity.

7. Ordinary kerosene to the extent of 0.25% by volume was added to trichloroethylene having an acidity of 17.0. After seven months the acidity was only 1.8.

I have found Nujol and higher boiling lubricating oils to be effective stabilizers but they have the disadvantage that they boil at high temperatures and therefore do not distill over with the trichloroethylene in effective amounts if that is the method of recovery. In general gasoline, either straight run or "cracked" and having boiling ranges between about 100° F. and 450° F. will be preferable. However, higher boiling hydrocarbon fractions, such as kerosene, are suitable for many purposes and also lower fractions having lower boiling limits than 100° F.

High-acid trichloroethylene is trichloroethylene that has suffered much decomposition and has a very high content of acidic substances. It has been found that the decomposition products auto-catalyze or promote the decomposition of trichloroethylene when present in very small quantities. The object of adding a few drops of high acid

trichloroethylene in examples 3 and 4 was to test the stabilizing effect of gasoline on trichloroethylene contaminated with decomposition promoters. The results show that gasoline is a good stabilizer under these conditions.

Gasoline may be added to the trichloroethylene before distillation or after distillation. Indeed, gasoline can be added whenever the trichloroethylene shows indications of increasing acidity. Thus, where this solvent is used for extraction or other purposes it may be advisable to add small amounts of gasoline from time to time to keep the trichloroethylene sweet by inhibiting further acid formation and reducing that already present.

This invention is not limited to any specific proportions of hydrocarbons and trichloroethylene. As little as 0.01% by volume of gasoline or similar liquid hydrocarbons will effect marked stability. For most practical purposes, however, it is necessary to have at least 0.025% and preferably over 0.05% by volume of stabilizer in the trichloroethylene. For certain purposes it is desirable to add as much as 50% or more of stabilizer in which case a mixture results having an exceedingly high acid stability and at the same time the flammability of the hydrocarbon fraction is greatly reduced.

The stabilizer may be any hydrocarbon material, single compound or mixture, that is liquid at room temperature and belonging to the aliphatic series. Either straight run or cracked gasoline may be used. In the claims the term "gasoline" is intended to cover any aliphatic hydrocarbon material within the boiling range of 100 and 450° F.

Claims:

1. Composition of matter comprising trichloroethylene and stabilizing amounts of gasoline.
2. Composition of matter comprising upwards of 90% trichloroethylene and the remainder aliphatic petroleum hydrocarbon material.
3. Composition of matter comprising upwards of 90% trichloroethylene and the remainder a petroleum hydrocarbon material having a boiling range between about 100° F. and 450° F.
4. Composition of matter comprising upwards of 90% trichloroethylene and the remainder gasoline.
5. Process of stabilizing trichloroethylene which comprises adding gasoline thereto.
6. Process of stabilizing trichloroethylene which comprises distilling trichloroethylene in contact with gasoline.
7. Process for reducing the acidity of trichloroethylene which comprises treating trichloroethylene with gasoline.
8. Process for reducing the acidity of trichloroethylene which comprises distilling trichloroethylene in contact with gasoline.

9. Composition of matter consisting of trichloroethylene and between about 0.01% and 50% by volume of gasoline.

Signed at Niagara Falls in the county of Niagara and State of New York this 7th day of January A. D. 1929.

CHARLES DANGELMAJER.

75

80

85

90

95

100

105

110

115

120

125

130